

# United States Patent

[19]

[11] 3,793,008

Tarshis et al.

[45] Feb. 19, 1974

[54] MONOCARBIDE FIBER-REINFORCED  
IRON-BASE SUPERALLOY COMPOSITE  
EUTECTIC CASTINGS AND METHOD

[75] Inventors: Lemuel A. Tarshis, Latham; Edward R. Buchanan, Burnt Hills, both of N.Y.

[73] Assignee: General Electric Company, Schenectady, N.Y.

[22] Filed: Mar. 1, 1972

[21] Appl. No.: 230,928

[52] U.S. Cl..... 75/128 G, 75/129, 75/130.5

[51] Int. Cl..... C22c 39/20

[58] Field of Search ..... 75/135, 128 G, 130.5, 129

[56] References Cited

UNITED STATES PATENTS

3,528,808 9/1970 Lemkey et al. .... 75/170

|           |        |                      |        |
|-----------|--------|----------------------|--------|
| 3,554,817 | 1/1971 | Thompson .....       | 148/32 |
| 3,564,940 | 2/1971 | Thompson et al. .... | 75/134 |
| 3,671,223 | 6/1972 | Thompson et al. .... | 75/122 |

Primary Examiner—L. Dewayne Rutledge

Assistant Examiner—E. L. Weise

Attorney, Agent, or Firm—Gerhard K. Adam; Joseph T. Cohen; Jerome C. Squillaro

[57] ABSTRACT

A high performance eutectic casting comprised of an iron-base alloy matrix reinforced with 8 to 19 volume percent of uniformly aligned fibers of a metal monocarbide extending continuously entirely through the casting is made by directionally solidifying a melt containing the constituents of the monocarbide in amounts corresponding to the monocarbide content of the eutectic. The solidification rate is at least  $\frac{1}{4}$  inch/hour.

7 Claims, 2 Drawing Figures

PATENTED FEB 19 1974

3,793,008

SHEET 1 OF 2

Fig. 1.



PATENTED FEB 19 1974

3,793,008

SHEET 2 OF 2

Fig. 2.



**MONOCARBIDE FIBER-REINFORCED IRON-BASE SUPERALLOY COMPOSITE EUTECTIC CASTINGS AND METHOD**

**FIELD OF THE INVENTION**

The present invention relates in general to iron-base alloy compositions, and more particularly to novel eutectic castings having iron-base alloy matrices which are reinforced by a fibrous phase of uniformly aligned fibers of a metal monocarbide extending continuously entirely through the castings. This invention is also concerned with a new method by which these novel castings can be produced.

In particular embodiments of this invention, these alloys have utility as directionally solidified castings forming gas turbine engine components.

**BACKGROUND OF THE INVENTION**

The physical and chemical requirements of materials of construction of gas turbine hot stage components have escalated since the advent of the aircraft jet engine because engine performance improvements require large operating temperature increases. For a long time, nickel-and cobalt-base alloys have served as the principal high-temperature materials of construction of jet engine buckets and vanes. The continual demand for materials of ever higher temperature capabilities has, however, resulted in the virtual exhaustion of alloying possibilities of the nickel-base and cobalt-base systems and has led to efforts to develop composite materials. While dispersion-strengthening of nickel- and cobalt-base alloys has not been promising, directional solidification of pseudobinary eutectics such as  $Ni_3Al$  or  $Ni_3Cb$  has resulted in somewhat improved high-temperature mechanical properties (Thompson and Lemkey, *Trans. ASM*, Vol. 62, page 140, 1969). Similar properties have also been obtained in the  $Ni-CbC$  system (Lemkey and Thompson, *Metal Trans.*, Vol. 2, page 1537, June, 1971) in which the typical directionally solidified body has a relatively ductile matrix strengthened by an aligned fibrous phase. In fact, the former eutectic has been used in the production of gas turbine buckets, the respective phases in these eutectic products being aligned to maximize physical properties in the desired location.

Limitations imposed by the simple pseudobinary eutectic alloy upon the properties of these directionally solidified composites were not avoidable until it was realized that the metal-monocarbide eutectics would withstand additions of alloying elements up to and somewhat beyond the point that the matrix qualifies as a high temperature iron-base alloy, i.e., an alloy characterized by deliberate additions of substantial amounts of nickel as an austenite stabilizer, chromium to improve elevated temperature environmental resistance and optional selective additions of cobalt, aluminum, molybdenum, tungsten, niobium, tantalum, titanium and yttrium to provide precipitation hardening capability, improved matrix solid solution strength or both. In these complex matrix chemistry alloys, we have further found that reinforcing monocarbide fibers can be derived from tantalum, titanium, niobium, zirconium, hafnium and vanadium, and from combinations of two or more of these elements with carbon. We provide carbon in these alloys in amount sufficient as a source of the metal monocarbide plus an amount in

equilibrium with the monocarbide in solution in the alloy matrix.

Additionally and very importantly, we have discovered that directionally solidified, monocarbide eutectic alloy castings which are free from structural inhomogeneity can be consistently produced. Thus, through critical control of the casting melt composition, one can in accordance with this invention make directionally solidified castings in which the fibrous monocarbide structure extends continuously from one end surface to another of an as-cast body. The necessity for trimming the casting to eliminate non-fibrous portions can thereby be avoided without incurring any offsetting penalty of cost or product performance capability. Moreover, this result can be obtained in castings of a variety of shapes and sizes with the continuous fibrous phase-forming capability being independent of casting dimensions and form.

**SUMMARY OF THE INVENTION**

This invention in both its method and article of manufacture aspects is predicated upon two basic novel concepts. First, we have found that engineering limitations such as oxidation and hot-corrosion tendencies can be avoided while retaining the metal-monocarbide fiber-reinforcing effects through additions of alloying elements to levels equivalent to and possibly beyond those of conventional alloys. Secondly, we have found that the metal-monocarbide fibrous reinforcing phase can be formed so that it is coextensive with a directionally solidified casting by providing a casting metal containing amounts of the monocarbide constituents corresponding to the monocarbide content of the eutectic.

Thus, broadly and generally, in its method aspect, this invention comprises the steps of preparing an iron base alloy casting melt containing, in addition to the alloy matrix chemistry, the metal-monocarbide constituents in amounts corresponding to the monocarbide content of the eutectic, and directionally solidifying the melt at the rate of at least  $\frac{1}{4}$  inch/hour. Determination of the amounts of the monocarbide constituents to be used in the formulation of the casting melt in accordance with this invention can be made experimentally, as will be subsequently described.

Likewise, broadly and generally, in its article aspect, this invention takes the form of an aligned composite cast eutectic body comprising an iron-base alloy matrix and a metal-monocarbide fibrous phase within the matrix providing reinforcement for the cast body. The fibrous phase consists essentially of aligned metal-monocarbide fibers extending continuously through the cast body from one surface to the other of the body in its original as-cast condition.

**DETAILED DESCRIPTION OF THE INVENTION**

The melt compositions provided according to this invention are iron-base alloys having a face-centered cubic crystal structure and containing at least 10.0 percent chromium and 5 to 14.0 percent of monocarbide-forming metals and 0.2 to 0.6 percent carbon. These compositions, as indicated above, may also contain substantial amounts of other metals as follows:

Cobalt — trace to 20.0 percent

Molybdenum — trace to 5.0 percent

Aluminum — trace to 8.0 percent

Titanium — trace to 5.0 percent

Yttrium — trace to 1.0 percent

Tungsten — trace to 5.0 percent

The volume fraction of metal monocarbide fiber in a composite eutectic casting of this invention depends upon the kinds and amounts of optional constituents of the alloy such as aluminum. Additionally, the metal-monocarbide content of the fibrous eutectic will be governed by the total composition, and particularly by the complexities of influences of constituents of the alloy on the composition of the eutectic. For these reasons, it is necessary to determine in some manner rather precisely the composition of the eutectic and the amounts of the monocarbide constituents of the eutectic so that the casting melt can be formulated.

One procedure which has been employed successfully involves preparation of an iron-base alloy casting melt in which the carbon and monocarbide-forming metal contents are well into the hypereutectic range. Directional solidification of this melt at a suitable rate such as  $\frac{1}{4}$  inch/hour results in an ingot or casting containing in some increment of its length the metal monocarbide fibers. Then, chemical analyses of that segment of the casting will yield the eutectic composition and consequently the formulation of another casting melt of this analyzed eutectic composition to be provided for directional solidification in accordance with the method of this invention to produce a new article of this invention.

The differences between the products of this invention and those resulting from the use of such hypereutectic casting melt are apparent from the drawings accompanying and forming a part of the specification, in which

FIG. 1 comprises a photograph of an as-cast ingot directionally solidified from a hypereutectic melt, and three photomicrographs (150 dia.) of microstructures in three different portions of one ingot as indicated; and

FIG. 2 comprises a photograph array corresponding to that of FIG. 1 in which the pictured ingot was produced in accordance with the invention by directional solidification of a casting melt containing the eutectic amounts of the monocarbide constituents.

10.0 percent nickel, 14.0 percent tantalum, 0.6 percent carbon and 55.4 percent iron. The composition of the matrix of this alloy is close to that of the cast stainless steel alloy, CF-3.

5 For purposes of comparison, an article of pure iron was produced by directional solidification, and a third article was likewise formed from an iron melt containing tantalum and carbon equivalent to 10.0 tantalum carbide.

10 The compositions of these four alloys are set out in Table I.

TABLE I

| Alloy     | Composition |      |      |       |      |
|-----------|-------------|------|------|-------|------|
|           | Fe          | Ni   | Cr   | Ta    | C    |
| FeTaC     | 90          | —    | —    | 9.7   | 0.3  |
| Fe        | 100         | —    | —    | —     | —    |
| FeCrNiTaC | 55.0        | 10.0 | 20.0 | 14.07 | 0.93 |
| CF-3      | 71.0        | 10.0 | 19.0 | —     | —    |

## EXAMPLE I

25 The casting designated in Table I as FeCrNiTaC was produced by directional solidification of a melt of identical composition at the substantially constant rate of  $\frac{1}{4}$  inch/hour in a temperature gradient of 250°C per inch.

Practically no segregation was found in the solidified 30 ingot, and the resulting microstructure had a matrix containing throughout substantially uniformly distributed and aligned monocarbide fibers, making up approximately 15.0 volume percent of the directionally solidified ingot. The fibers were essentially single crystal monocarbides each containing essentially carbon and tantalum. The matrix corresponded in composition to stainless steel containing chromium and nickel and small amounts of tantalum and carbon essentially in equilibrium with the fibers. The tensile properties of 35 this alloy, as well as those of pure iron and the other two alloys of Table I, tested at a strain rate of  $4 \times 10^{-2}$ /min., are listed in Table II for room temperature and in Table III for elevated temperatures.

TABLE II

| Alloy     | Room Temperature Tensile Tests |                             |              |
|-----------|--------------------------------|-----------------------------|--------------|
|           | 0.2% Yield Stress (psi)        | Ult. Tensile Strength (psi) | % Elongation |
| FeTaC     | 59,000                         | 60,000                      | 20.0         |
| Fe        | 14,000                         | 25,000                      | 48.0         |
| FeCrNiTaC | 90,000                         | 107,300                     | 53.4         |
| CF-3*     | 37,000                         | 77,000                      | 55.4         |

\* From reference work

TABLE III

| Alloy     | Test Temp. (°F) | Elevated Temperature Tensile Tests |                             |          |
|-----------|-----------------|------------------------------------|-----------------------------|----------|
|           |                 | 0.2% Yield Stress (psi)            | Ult. Tensile Strength (psi) | % Elong. |
| FeTaC     | 1200            | 27,000                             | 28,000                      | 14       |
| Fe        | 1200            | 2,000                              | 4,000                       | 72       |
| FeCrNiTaC | 1832            | 36,500                             | 37,000                      | 4.0      |
| CF-3      | 1832            | (2,000)                            | (4,000)                     | (50)     |

An article or product of the present invention is produced by directional solidification of a casting melt consisting essentially of about: 20.0 percent chromium,

The stress-rupture properties at elevated temperature of a typical article of this invention and of a typical stainless steel body are set out in Table IV.

TABLE IV

| Elevated Temperature Stress-Rupture Properties |              |                 |                           |
|------------------------------------------------|--------------|-----------------|---------------------------|
| Alloy                                          | Stress (psi) | Test Temp. (°F) | Life<br>(hrs. to rupture) |
| FeCrNiTaC                                      | 20,000       | 2000            | 1.3                       |
| CF-3                                           | 20,000       | 1375            | (1.3)                     |

As may be seen from the data of Tables II, III and IV, the metal monocarbide-reinforced iron-base eutectic alloys of the present invention has significantly superior high-temperature stress-rupture resistance and tensile strength from room temperature to 1,832°F, as compared to iron and stainless steel and tantalum carbide-reinforced iron bodies prepared as described in the following examples:

#### EXAMPLE II

The casting designated in Table I as FeTaC was produced by directional solidification of a melt of the composition stated in Table I in the manner described in Example I. In this directionally-solidified body, as in that of Example I, the monocarbides were in the form of aligned, uniformly dispersed TaC fibers throughout the iron-base alloy matrix, generally as illustrated in FIG. 2. These fibers made up about 18.7 volume percent of the directionally-solidified ingot.

#### EXAMPLE III

A melt of pure iron was cast in the conventional manner (not directionally solidified) to produce an ingot having no second phase.

Herein and in the appended claims proportions or percentages are stated on the weight basis unless otherwise expressly specified.

It will be obvious to those skilled in the art upon reading the foregoing disclosure that many modifications and alterations in the specific compositions and microstructures disclosed as non-limiting examples may be made within the general context of the invention, and that numerous modifications, alterations and additions may be made thereto within the true spirit and scope of the invention as set forth in the appended claims.

What we claim as new and desire to secure by Letters Patent of the United States is:

1. The method of forming a high performance eutectic casting comprising an iron-base alloy matrix with 8 to 19 volume percent of a fibrous phase consisting essentially of aligned fibers of a metal monocarbide and

extending continuously entirely through the casting in its ascast condition, which comprises the steps of preparing an iron-base alloy casting melt containing constituents of the monocarbide in amounts corresponding to the monocarbide content of the eutectic, and directionally solidifying said melt at a rate of at least  $\frac{1}{4}$  inch/hour.

2. The method of claim 1 in which the monocarbide is essentially TaC.

3. The method of claim 1 in which the casting melt consists essentially of about 55 percent iron, 20 percent chromium, 10 percent nickel, 14 percent tantalum and 0.6 percent carbon.

4. An aligned composite cast eutectic body comprising an iron-base alloy matrix and a metal-monocarbide fibrous phase within the matrix providing reinforcement for and imparting increased high-temperature stress-rupture life to the cast body, said fibrous phase

consisting essentially of aligned metal-monocarbide fibers and extending continuously through the cast body from one surface to another of said body in its original cast condition.

5. A cast body as described in claim 4 in which the body is elongated and the fibrous phase extends longitudinally of the body from one end face to the other of the casting.

6. The cast body of claim 4 which is a jet engine turbine bucket.

7. The composite cast body of claim 4 of composition within the following percent ranges:

chromium — 10.0 — 25.0

cobalt — trace — 20.0

aluminum — trace — 8.0

titanium — trace — 5.0

carbon — 0.2 — 0.6

monocarbide — 5.0 — 14.0 forming metal

tungsten — trace — 5.0

molybdenum — trace — 5.0

yttrium — 0.2 — 0.8

\* \* \* \* \*

UNITED STATES PATENT OFFICE  
CERTIFICATE OF CORRECTION

Patent No. 3,793,008 Dated February 19, 1974

Inventor(s) Lemuel A. Tarshis and Edward R. Buchanan

It is certified that error appears in the above-identified patent and that said Letters Patent are hereby corrected as shown below:

Column 6, claim 7, line 47, "monocarbide - 5.0 - 14.0 forming metal"  
should read --monocarbide - 5.0 - 14.0 --.  
forming metal

Signed and sealed this 18th day of February 1975.

(SEAL)  
Attest:

RUTH C. MASON  
Attesting Officer

C. MARSHALL DANN  
Commissioner of Patents  
and Trademarks